

# UNITED STATES PATENT OFFICE.

LUDWIG KERN, OF HAMBURG, GERMANY.

## PROCESS FOR PRODUCING ARTICLES FROM DIATOMACEOUS EARTH.

Specification of Letters Patent. Patented Nov. 28, 1916.

1,206,546.

No Drawing.

Application filed May 15, 1915. Serial No. 23,309.

To all whom it may concern:

Be it known that I, LUDWIG KERN, a subject of the German Emperor, residing in Hamburg, Germany, have invented a new and Improved Process for Producing Articles from Diatomaceous Earth, of which the following is a full, clear, and exact description.

The invention relates to the ordinary diatomaceous earth of a low quality and incapable of being molded into shape, and such as is found in large quantities in various parts of the world.

The object of the invention is to provide a new and improved process for making diatomaceous earth moldable, without the use of clay, for producing various industrial articles such, for instance, as are used for filtering or purifying liquids and gases, 20 diaphragms for use in electro-chemistry for the separation of the anode and cathode spaces, fire bricks for use in kilns, smelting and other furnaces, as insulating material for electricity, heat, sound and fire, or for 25 building or other purposes.

In order to accomplish the desired result, a diatomaceous earth of low quality is subjected to the action of a diluted mineral acid such as hydrochloric acid to disintegrate the 30 carbonates of iron, calcium, sodium, magnesium, potassium and the silicates usually found as extraneous matter with the said diatomaceous earth. By the action of a mineral acid a mass is formed which is free 35 of carbonates and capable of being molded into a desired shape, to be finally burned with a view to produce an article of compressional strength. By the use of the mineral acid the carbonic acid of the carbonates is driven off and corresponding salts 40 dissolvable in water are formed. The process can be carried on cold, but by the use of heat the time for carrying out the process can be materially shortened. The diatomaceous earth itself is not affected by this 45 process and practically remains intact, but a number of salts dissolved in water are produced which are of a viscous character and are minutely distributed in the hereinbefore mentioned salt solution, which renders the diatomaceous earth plastic and capable of being readily molded into any desired shape. After the article is formed it is burned in a suitable oven and during 50 the burning and oxidizing operation, the

salts form a liquid flux for producing a hardening of the material.

In carrying out the process in detail, I proceed as follows: A desired amount of raw diatomaceous earth of the character described is placed in a mixing vessel and then diluted mineral acid is added to cause a disintegration of the basic substances contained in the diatomaceous earth and form therewith a thick moldable paste. As the 65 extraneous substances in the raw diatomaceous earth vary considerably, both in nature and in quantity, it is desirable, first, to obtain by laboratory tests the necessary data for carrying out the process on a 70 large scale, that is, for enabling the operator to determine the properties of the mineral acid to be used for any particular batch of diatomaceous earth. In some of the 75 deposits of diatomaceous earth the extraneous substances are of low percentage and as the strength of compression of the final product depends to a considerable extent on the extraneous substances, it is necessary in some 80 cases to add such substances to the diatomaceous earth contained in the mixing vessel.

After the paste is formed, it is left to stand for a short time, say 6 to 24 hours and then it is placed into suitable molds corresponding to the article to be made. The 85 molded article is then partly dried so that quite a percentage of the water is retained, and then the molded article is burned in a suitable oven or furnace. During the burning process the heat of the firing gases causes 90 the water in the molded article to be converted into hydrogen and oxygen. The hydrogen forms with the chlorin of the chlorid, hydrochloric acid, which escapes together with the iron chlorid, it being understood that this process is facilitated by the incandescence of the article. The oxygen forms the oxid of potassium, magnesium and sodium, thereby forming a 95 liquid flux which is minutely divided in the mass of the diatomaceous earth and causes a hardening of the same. The article produced in the manner described is insoluble in cold or boiling water, has a hard sound, can be cut, bored, sawed or nailed, and is very porous.

The diluted mineral acid consists preferably of about 1,000 parts of water and from 5 to 50 parts of the hydrochloric acid or other mineral acid. The amount of min-

eral acid depends on the nature, quality and amount of the extraneous substances contained in the diatomaceous earth. The amount of the mineral acid is about 100 to 250 parts to 100 parts of the diatomaceous earth and the mixture is carried on under normal temperature.

Having thus described my invention, I claim as new and desire to secure by Letters 10 Patent:

A process for the production of articles from diatomaceous earth containing acid soluble metal compounds, which consists in mixing the diatomaceous earth and its com-

pounds with diluted hydrochloric acid to 15 convert the compounds into chlorids and to form a moldable mass, then molding the mass and partly drying the same, and then burning the molded product to transform the chlorids of the compounds into oxids. 20

In testimony whereof I have signed my name to this specification in the presence of two subscribing witnesses.

LUDWIG KERN.

Witnesses:

FRANCIS R. STEWART,  
CHARLES A. HALLEY, JR.